

## UNITED STATES PATENT OFFICE

2,337,478

## LUBRICANT

Bert H. Lincoln, Ponca City, Okla., and Gordon D. Byrkit, Niagara Falls, N. Y., assignors, by mesne assignments, to Socony-Vacuum Oil Company, Incorporated, New York, N. Y., a corporation of New York

No Drawing. Original application March 14, 1940, Serial No. 323,960. Divided and this application April 15, 1942, Serial No. 439,094

1 Claim. (Cl. 252—51)

This invention has to do with the improvement of lubricants and is more particularly concerned with lubricant compositions which have been improved in various characteristics, such as resistance to oxidation and to the formation of corrosive products during use, by the incorporation therein of a minor proportion of a characterizing ingredient. This application is a division of our copending application Serial No. 323,960, filed March 14, 1940, now Patent Number 2,297,658, issued September 29, 1942, which in turn was a continuation-in-part of our application Serial No. 231,362, filed September 23, 1938.

Present-day mechanical devices require lubricating oils of high film strength, of high oiliness characteristics, and of low tendency to oxidize during use. It has been found that the present-day hydrocarbon lubricants of the very highest quality are deficient in these very important characteristics. These three properties are of vital importance under conditions of thin film lubrication where the lubricant has been squeezed from between the friction surfaces because of high pressure, slow speeds, and other causes. It is readily seen that the viscosity or the body of the lubricant plays no part in this type of lubrication and that the remaining film of oil must have a very high film strength and be of high oiliness value to prevent rupture of the film of the lubricant, which would cause seizure. The oil film must tend to keep the coefficient of friction as low as possible. The oil must resist oxidation when these thin films are heated in the presence of oxygen as they are in use.

Mechanical devices are being designed for higher pressure operation, and the film strength of the best quality straight hydrocarbon lubricant has been found to be too low. It will be obvious that an invention which provides a means of improving the film strength of these lubricants is of great importance to the art of lubricant manufacture and to the designer and fabricator of mechanical devices.

Substantially all machines operate in part or at times totally under conditions of boundary or thin film lubrication, under which conditions the oiliness or unctuousness of the lubricant is the first and primary requisite of efficient operation. Those skilled in the art of lubricant manufacture or machine manufacture will readily appreciate the value of an invention that will improve the oiliness of these otherwise high-quality lubricants. Furthermore, sludge and acid are especially deleterious under conditions of thin film lubrication. The sludge is not a lubricant in any sense of the word, and the soluble acid is particularly corrosive to bearing metals such as cadmium-silver, copper-lead, and the like.

In starting idle mechanical equipment which is lubricated from a sump by pumping or circulating the lubricant, there is always a short period of time in which the rubbing surfaces must operate under conditions of dry friction if ordinary hydrocarbon lubricants are used. With dry friction, the wear on friction surface is extreme; and during cold weather when the lubricant is sluggish or during periods when the lubricating system is not functioning properly for one reason or another, rubbing surfaces may not only suffer considerable wear but may be damaged to the point where they must be replaced. The product of our invention has a very important property of reacting with the metal surfaces, penetrating or adsorbing on the metal surfaces, and leaving a film of lubricant with high oiliness character, which remains on the metal surface irrespective of the length of time the machine has been idle.

This high oiliness film gives very even and smooth operation, which may be easily discerned by the experienced operator or lubricating engineer.

When the hydrocarbon lubricants are diluted with unburned fuel or with other light hydrocarbons, the small degree of oiliness of the original hydrocarbon lubricant is greatly decreased. We have found that the addition of the products of our invention to hydrocarbon lubricants more than compensates for the loss in oiliness and load-carrying ability from dilution.

It is well known that, in order to obtain lubricants which are preeminently satisfactory from the standpoint of oxidation in use, it is necessary to refine the oil thoroughly and then to add an inhibitor of oxidation. The thorough refining may consist of more and heavier acid treatments or solvent treating so as to remove a considerable part of the oil and leave only the most stable portion. Such drastic refining is necessary in order to obtain stability with respect to sludge formation, but the oil is then subject to easy oxidation to form soluble acids and other corrosive materials. This can be prevented by the addition to the refined oil of small amounts of materials which either prevent the formation of these corrosive products or by the same action render them inert. Furthermore, such well-refined oils are susceptible to the formation during use of lacquerlike materials which tend to stick rings. This results in a blow-by and hence loss of power, failure of lubrication, scratching, scoring, overheating, and eventually replacement of parts. It is practically impossible to refine a lubricant in such a manner as to avoid all three of these difficulties, namely, sludge, soluble corrosive products, and lacquer. It is considerably

more advantageous to add the materials of our invention and avoid these difficulties by this method.

Many of these additive materials are effective when added to poorly refined or even wholly unrefined lubricants. The addends may thus be substituted in whole or in part of the usual refining processes.

In the prior art of applying these principles to the manufacture of lubricants, many diverse types of materials have been suggested to be added to obtain improvement in various characteristics. It has been found that the addition of various organic esters of the oxygen and sulfur acids of phosphorus frequently improves film strength, oxidation, resistance, non-corrosiveness, and other characteristics. Nitrogen compounds have been found to inhibit oxidation of oils. Our materials combine both of these properties.

One object of our invention is to provide improved inhibitors of oxidation and corrosion for addition to lubricants.

Another object of our invention is to provide film strength improving addition agents suitable for use in lubricants and especially in crankcase lubricants.

Other and further objects of our invention will appear in the course of the following description.

In general, our invention involves the use of certain organic arsenic compounds containing at least one arsenic-nitrogen bond to hydrocarbon fuels and lubricants. We have discovered that these materials which may be broadly characterized as arsenical derivatives of aromatic amines combine the advantages of phosphorus compounds and nitrogen compounds and are frequently even more effective in preventing the development of corrosive materials in the oil during use than their nitrogen and phosphorus analogues.

The present invention is particularly concerned with the arsenical derivatives of aromatic amino ethers or the arsen-aryl amino ethers as oil-improving agents. The general class of arsen-aryl amino ethers contemplated herein may be represented by the general formula:



in which R represents an aromatic or an alkyl-substituted aromatic radical; n is the integer one or two and R' represents an organic radical. Of the general class of ethers represented by the foregoing formula, preference is given to the diethers corresponding to the general formula  $RNHAs(OR')_2$  in which R and R' have the same significance defined above. Listed below are several representative examples of compounds of the type contemplated herein. All and each of these are to be considered as examples of our invention when blended in an oil of lubricating viscosity.

#### Examples

- (1) Arsen-anilino dimethyl ether  
 $C_6H_5NHAs(OCH_3)_2$
- (2) Arsen-toluidino dicresyl ether  
 $CH_3C_6H_4NHAs(OC_8H_4CH_3)_2$
- (3) Arsen-p-tert.-butyl anilino dilauryl ether  
 $C_4H_9C_6H_4NHAs(OC_{12}H_{25})_2$
- (4) Arsen-anilino dibenzyl ether  
 $C_6H_5NHAs(OCH_2C_6H_5)_2$

Any of these compounds or other members of the classes represented or their derivatives with-

in the limitations set forth above may be used within the scope of our invention.

It is to be understood that in practicing our invention, oil-soluble organo-arsenic-nitrogen ether compounds of the type described are to be selected. Some of the examples described have only limited solubility in hydrocarbon oils. It is to be remembered, however, that, because of their great efficiency, extremely small amounts are often effective. Thus, we may use as little as 0.001 per cent of some of these compounds, and it will be seen that a fairly insoluble material may dissolve to a sufficient extent to be satisfactory for our purpose. In general, more than 0.001 per cent of our addition agents are used, and we may add one, two or even five per cent or more.

Furthermore, it is well known that different types of oils have different capabilities of dissolving a given material. For some purposes, therefore, we prefer paraffinic lubricants, while for other purposes we prefer naphthenic or mixed base lubricants. Another method of obtaining a satisfactory mixture of addition agent with the hydrocarbon oil is the use of a mutual solvent to bring the addend into solution. Alternatively, peptizing agents may be added to maintain the organo-arsenic compound in permanent suspension.

Many of the more difficultly soluble materials are rendered more soluble by the introduction of alkyl groups, particularly those containing four or more carbon atoms. The iso-amyl, octyl, lauryl, and octadecyl radicals and radicals from paraffin wax greatly increase the solubility of organic compounds in oil. One or more of such groups may be introduced as required into the previously described compounds or their derivatives. For example, arsen-anilino dimethyl ether is not very soluble in hydrocarbon lubricating oils but arsen-p-tert.-butylanilino dilauryl ether is much more soluble.

The selection of a particular compound or compounds to be used as an addition agent to the hydrocarbon oil is more or less dependent upon the use to which the blend is to be put. Thus, if water is likely to be present during use, an arsen-aryl amino ether compound or combination of compounds is selected which is not affected by water. In general, we prefer to use compounds having boiling points over 250° F. It is sometimes advantageous to combine more than one of these compounds in a blend to obtain particular properties. We accomplish this by mixing two or more of these compounds together and blending the mixture with the hydrocarbon oil or by blending one in the hydrocarbon oil, blending the second into this mixture, and so on until the composition is complete.

The various arsen-aryl amino ether compounds contemplated herein usually improve both the film strength and oxidation characteristics of the hydrocarbon oil. For example, the sludging tendencies may be decreased by as little as 0.001 per cent of the arsen-aryl amino ether compounds. The oxidation characteristics of lubricants are very important, and these are markedly improved by minor proportions of our compounds. The ability to reduce friction is another feature contributed to lubricants by small amounts of our arsenic-nitrogen compounds.

It may be desirable to include in one and the same blend based on a hydrocarbon oil, in addition to the addends here described, other addends

for specific purposes. Thus, we may add a pour point depressor such as a naphthalene-chlorwax condensation product and a viscosity index improver such as certain resins or polymerized hydrocarbons in addition to our organo-arsenic compounds. Furthermore, various other metallic compounds may be added to the blend without interfering with the action of our ingredients. Indeed, in some cases, it is advantageous to combine with our organic arsenic-nitrogen compounds in a hydrocarbon oil blend such materials as calcium dichloro-stearate, chromium oleate, tin octadecyl phthalate, aluminum stearate, and other metallic soaps.

Our addends are admirably adapted for use in lubricating oils of all types including those designed for use in automotive crankcases, Diesel oils, and any other oils of lubricating viscosity such as castor oil, cotton seed oil, lard oil, sperm oil, shale oil. Furthermore, our addends are advantageously blended in gasoline and other petroleum fuels, either directly or after being blended first in a lubricating oil and then added to the fuel. Soap-thickened mineral oils of all types ranging from those showing only a slight increase in viscosity over that of the mineral oil alone to the semi-solid and solid greases containing fifty per cent or more of soap are amenable to treatment according to our invention. In making these greases, the usual soaps such as sodium stearate, aluminum stearate, calcium soaps of beta fat and the like may be used. Various other thickening ingredients or materials for other purposes may be added. These include yarn, hair graphite, 35

glycerol, water, lamp black, mica, zinc dust, litharge, and the like.

The following example illustrates one type of lubricant composition in which improving agents 5 of the type contemplated herein may be used. It is to be understood, of course, that this example is merely illustrative and in no way limits the scope of the invention because, as aforesaid, the arsen-aryl amino ethers may be used 10 with or without other addends in the oil composition.

*Example*

|                                             | Per cent |
|---------------------------------------------|----------|
| Paraffin base bright stock                  | 57.0     |
| Paraffin base neutral stock                 | 40.0     |
| Sulfurized methyl esters of corn oil esters | 1.1      |
| Arsen-anilino dimethyl ether                | 0.2      |
| Calcium dichloro-stearate                   | 1.3      |
| Diphenyl-chlorwax condensation product      | 0.4      |

The arsen-aryl amino ether may be used in the oil fraction in a small amount varying from 0.001 to 1.0 per cent or more and it is to be understood that while we have illustrated this invention with certain specific compounds and with a typical lubricant composition, the invention is not limited to the examples given but includes within its scope whatever changes fairly come within the spirit of the appended claim.

We claim:

30 A lubricant comprising in combination a major proportion of oil of lubricating viscosity and a minor proportion of arsen-anilino dibenzyl ether.

BERT H. LINCOLN,  
GORDON D. BYRKIT.